

3,219,465

## FOUNDRY MOLD COATING

Phillip F. Herkimer, Royal Oak, Neil M. Lottridge, Jr., Warren, and Douglas G. McCullough, Rochester, Mich., assignors to General Motors Corporation, Detroit, Mich., a corporation of Delaware  
No Drawing. Filed May 26, 1961, Ser. No. 112,755  
7 Claims. (Cl. 106—38.23)

This invention relates to a coating composition, which when applied to foundry sand mold and core surfaces, functions as an effective anti-veining coating to appreciably improve the surface finish of castings produced by the use of such a mold or core. In addition, the fluidity of molten casting metals, such as gray cast iron, malleable iron, spheroidal graphite cast iron, aluminum alloys and magnesium alloys, poured into contact with the coated mold or core is significantly increased. More specifically, the invention pertains to a foundry mold or core wash containing finely divided mica, corn cereal and wood flour suspended in a liquid carrier.

In the past it was frequently impossible to successfully cast some thin sections of the aforementioned metals except by superheating the casting metal, preheating the mold and/or substantially increasing the metallostatic pressure. Obviously it is desirable to eliminate these procedures. A principal object of the present invention, therefore, is to provide a coating for foundry sand molds and cores which materially increases the fluidity of molten casting metals contacting such molds and cores without employing superheat, preheated molds or undesirably high metallostatic pressures. As a consequence, sound castings of very thin section can be formed by conventional procedures. The term "fluidity," as used herein, refers to that property of molten casting metal in contact with a mold which allows the metal to flow into the mold and fill it before solidification obstructs further flow of the metal.

The above and other objects of this invention are attained with a foundry mold and core coating comprising a slurry of mica or vermiculite powder, powdered corn cereal, wood flour and a liquid vehicle, such as methyl alcohol, ethyl alcohol, isopropyl alcohol, toluene, a chlorinated hydrocarbon, commercial mineral spirits or water. Small amounts of a suspension agent, a binder, a low-foaming, nonionic wetting agent and an antifermmentation agent also may be beneficially included in the slurry. The coating composition thus provided is relatively inexpensive and can be readily applied to the mold surfaces by conventional means, such as spraying, dipping or brushing.

It will be understood that the term "mold," as hereinafter generally employed, means a casting form which includes both molds and cores, this invention not being limited to the former. Likewise, the word "sand" is used in its generic sense and is not restricted to silica particles.

This mica powder should constitute about 70% to 95% by weight of the solids content of the coating composition, while the amount of corn cereal to be used may vary from approximately 2% to 20% of the weight of the solids. In general, the wood flour content can range between about 1% and 12%. The preferred solids composition includes approximately 75% to 90% by weight of mica powder, 4% to 14% by weight of corn cereal and 3% to 8% by weight of wood flour. For most applications the particle sizes of these powdered constituents should be between —80 and —325 mesh, although finer powders may be used.

The presence of the corn cereal permits the slurry to be handled more conveniently than the mold coatings

heretofore proposed for the same purpose. This is possible because of the lower liquid-to-solids ratio permissible with the new coating composition and the resultant faster drying time. The suspension is easier to apply to molds and cores, particularly by dipping, and its superior consistency reduces the amount of coating material lost due to dripping. Also, a smaller amount of wetting agent can be employed, and the wetting agent may be eliminated entirely for some applications. In addition, the presence of corn cereal permits a reduction in wood flour content with a consequent decrease in the amount of mold gas generated during pouring of the molten casting metal. As a result, the castings are sounder and less porous.

The coating slurry preferably is applied to green sand molds by a spraying procedure, and when this is done it is advantageous to mix the above-described powdered constituents with a volatile organic liquid, such as commercial methyl alcohol, ethyl alcohol, isopropyl alcohol, toluene, a chlorinated hydrocarbon or naphthol spirits. A slurry of this type also can be used to spray baked sand molds and cores, or water may be employed as a less expensive carrier if the molds and cores are subsequently reheated to dry the coating. Of course, in the case of baked sand cores, it is convenient to apply a water slurry by a dipping operation. When alcohol is used as the liquid carrier, any excess alcohol can be readily burned off.

In order to obtain a proper dispersion of the coating composition on the mold surfaces when a water suspension is used in a dipping operation, it is desirable to include a wetting agent. A low-foaming, nonionic wetting agent is preferred. Examples of such a wetting agent are those available under the trade names "L-62 Pluronic" and "L-64 Pluronic." Likewise the adherence of the coating to the mold may be further improved for some applications by adding a thickener or binder to the slurry. Methyl cellulose has proved to be a satisfactory water thickener, but other short-chained alkyl celluloses, such as ethyl cellulose, butyl cellulose and propyl cellulose, may be employed. "Ceron N-4S" also has proved to be an excellent suspension agent and binder. This water-soluble derivative of wheat starch is a nonionic, etherified polymeric carbohydrate. A water thickener of this type appreciably improves the dipping characteristics of the slurry and increases the hardness and durability of the dried coating.

The amount of liquid carrier used should be sufficient to provide a slurry which can be readily applied to the mold. If it is desired to dip the mold, the ratio of the liquid carrier to the solids content of the coating composition may vary between approximately 4 to 1 and 10 to 1. On the other hand, this ratio may be as low as 2 to 1 for spray coatings. Thus it will be seen that the amount of liquid in the slurry may constitute about 65% to 91% of the total weight of the slurry, but a coating having a water content of approximately 75% to 85% is generally preferred.

When a wetting agent is used in the mixture, the addition of 0.5 gram to 2 grams of this material to 500 milliliters of slurry has proved to be adequate. In fact, as little as about 0.1% by weight of wetting agent improves the coating composition, and as much as 1% wetting agent sometimes may be used to advantage. Dipping characteristics and slurry suspension are further improved when the composition contains "Ceron N-4S" in an amount equal to about 1% to 5% by weight of the solids in the composition. Approximately 2 to 3 grams of this material added to 500 milliliters of the slurry has proved to be particularly effective. When methyl

cellulose is used it preferably constitutes approximately 0.2% to 1% by weight of the solids in the slurry.

In addition to the above-described constituents, urea formaldehyde or other soluble resins may be included in the slurry, particularly if a wetting agent is to be used, to further increase the hardness and durability of the dried coating. A relatively small amount of other binder materials also may be added to the slurry to improve the adhesion of the coating to the sand mold if the binder is soluble in the liquid carrier. Among 10 these binding agents are thermoplastic resins such as polyvinyl chloride, vinylidene chloride, polyvinyl alcohol

5 agitated. In general, it is desirable to maintain the pH of the water between 5 and 7 because some of the solid constituents appear to disperse somewhat better in water which is slightly acidic. If urea formaldehyde is to be included in the coating, it is the last constituent added to the slurry. The coating composition should be stirred for several minutes and not used for at least four hours. Normally it is applied to the casting-defining surfaces of the mold at room temperature.

10 The following table lists specific examples of coating compositions prepared in accordance with the present invention:

|                                      | Example I | Example II | Example I | Example IV | Example V |
|--------------------------------------|-----------|------------|-----------|------------|-----------|
| Water                                | 100 gal   | 40 gal     | 500 ml    |            | 800 ml.   |
| Isopropyl alcohol                    |           |            |           | 300 ml     |           |
| Mica powder (-160 mesh)              | 100 lb    | 58.5 lb    | 80 gm     | 88.5 gm    | 85 gm.    |
| Corn cereal                          | 11 lb     | 3.4 lb     | 10 gm     | 5 gm       | 10 gm.    |
| Wood flour (-80 mesh)                | 5.6 lb    | 3.4 lb     | 10 gm     | 5 gm       | 5 gm.     |
| Wetting agent                        | 300 gm    | 40 ml      | 1 gm      |            | 1 gm.     |
| Ceron N-4S thickener                 | 4 lb      | 1.67 lb    |           |            | 4 gm.     |
| Calcined clay                        |           |            | 1 gm      |            |           |
| CuSO <sub>4</sub> ·5H <sub>2</sub> O | 0.24 lb   | 60 gm      |           |            | 0.2 gm.   |
| Phenol-formaldehyde resin            |           |            |           | 2.5 gm     |           |

30 and polyvinyl acetate, and thermosetting resins such as phenolformaldehyde and melamine formaldehyde. Of course, various other binders besides the polymeric vinyl and phenolic resins can be employed. For example, linseed oil and certain clays, such as bentonite clay, are useful as binder constituents.

35 When a coating composition having mineral spirits or alcohol as the carrier is to be applied by spraying, certain thermoplastic, lignin-type resinous materials derived from wood and containing both methoxyl and hydroxyl groups have proved to be useful as additional binders if included in the slurry in small amounts. Such materials may be obtained from a variety of wood products, including sawdust, waste liquor from the paper industry, wood chips, etc., by physical and/or chemical treatment. Illustrative of one type of thermoplastic resinous material is a substantially gasoline-insoluble resinous material obtained by extracting a resinous wood with a coal tar hydrocarbon, removing the hydrocarbon by evaporation, leaving a residue comprising a mixture of wood rosin and thermoplastic resinous material, and extracting the rosin with a petroleum hydrocarbon, leaving a thermoplastic resinous material. Such a product is available under the trade name "Vinsol."

40 Of course, more than one binder may be used in the coating composition, but the total binder content in addition to the corn cereal normally should not constitute more than about 5% of the weight of the solids in the coating material. Even 0.5% by weight of the additional binder in the coating causes it to adhere more 45 strongly to the mold.

45 A water slurry containing wood flour, corn cereal and/or "Ceron N-4S" will ferment after a relatively short time, thereby reducing the bonding action of the Ceron N-4S and the corn cereal. Hence, we have found it desirable to include a small amount of an antifermentation agent to retard the growth of bacteria. Copper sulfate, potassium chromate, sodium chromate, sodium hyperchlorate, urea formaldehyde and paraformaldehyde all have proved to be useful for this purpose. Shelf life of an aqueous slurry has been increased from approximately 3 days to more than 2 weeks because of the antibacterial action of such an additive.

50 The above-described coating slurry may be prepared in the following manner: The dry materials, such as the mica, corn cereal and wood flour, are preferably first blended to powder form. Next, the wetting agent is added to the desired amount of water, assuming an aqueous slurry is to be used; and the blended solids are introduced slowly into the slurry while the latter is being

55 Each of the above coating compositions had excellent dipping characteristics, dried in a reasonable period of time and was hard and durable upon drying. In addition, the coatings substantially reduced chill in thin sections and materially aided in the cleanup of the castings. Furthermore, use of these coatings as compared with currently commercially used green sand mold sprays and core washes significantly decreased metal penetration into the mold and/or cores, thereby improving the surface finish of the castings in their as-cast condition.

60 When dry sand test molds were coated with the above-described slurries, the fluidity of gray cast iron, malleable iron and spheroidal graphite cast iron poured at normal casting temperatures into these molds was increased more than 100% as compared with similar molds which were uncoated. The fluidity of the molten metals in the molds was determined by means of a double spiral fluidity test mold in which one spiral is coated with the mold wash while the other remains uncoated, both being fed by the same pouring basin and down sprue. The relative distances the metal travels in the spiral is a measure of the improvement in fluidity. This test mold design and the procedure for using it are described in Transactions of the American Foundrymen's Society, volume 67, (1959), pages 496 to 507.

65 Tests have been conducted on castings of gray iron, malleable iron, spheroidal graphite cast iron and aluminum alloys which were formed in molds coated in accordance with this invention. As a result of these tests, it was found that these metals could be successfully cast in thin sections by using the above-described mold wash and that the resultant castings all had exceptionally high ultimate tensile strength and hardness.

70 For example,  $\frac{1}{8}$ -inch thick sections of gray iron cast in green sand mold portions coated with this mold wash were compared with gray iron specimens of the same composition from  $\frac{3}{16}$ -inch thick sections cast in the same molds without a coating. The cast iron in the  $\frac{1}{8}$ -inch thick sections had appreciably higher ultimate tensile strength and hardness than the cast iron in the  $\frac{3}{16}$ -inch thick sections. Attempts to cast  $\frac{1}{8}$ -inch thick sections without first coating the surfaces of the mold cavities were unsuccessful because the molten metal would not properly feed into and fill the narrow mold cavities. The gray cast iron which did feed into these  $\frac{1}{8}$ -inch cavities of uncoated molds was chilled, and hence these portions of the castings were hard, brittle and unmachinable. Green sand molds, each having two cavities four inches wide and 18 inches long, with sections  $\frac{1}{8}$ -inch and  $\frac{3}{16}$ -inch deep, were used in these tests.

It was further noted that the microstructure of the  $\frac{1}{8}$ -inch thick sections of gray iron castings poured into the coated mold portions was slightly more refined than the microstructure of gray iron specimens cast into the  $\frac{3}{16}$ -inch thick uncoated portions of the same mold. No primary carbide was evident in either section.

Additional tests under production conditions also showed that use of the new mold coating improved the surface finish of the castings and decreased the incidence of veining, thus greatly reducing the amount of labor necessary in cleaning operations. Moreover, the coating prevented misruns and cold shuts. As a consequence, leakers were eliminated, and the scrap rate due to such defects was lowered from approximately 9% to less than 1%. Furthermore, the mold coating described herein has a relatively short drying time and a wide drying temperature range. It may be dried at a temperature up to approximately 500° F. without blistering and coatings on port cores for gasoline engine cylinder head castings were dried in only about five minutes at 500° F. This coating composition also has good dipping characteristics and is uniform in thickness both before and after drying, as well as being relatively inexpensive to use.

While our invention has been described by means of certain specific examples, it is to be understood that its scope is not to be limited thereby except as defined by the following claims.

We claim:

1. A slurry for coating casting-defining surfaces of foundry sand molds, said slurry being formed from a dry blend consisting essentially of about 70% to 95% by weight of mica powder, about 2% to 20% by weight of corn cereal and about 1% to 12% by weight of wood flour to which has been added a liquid carrier in an amount sufficient to constitute about 65% to 91% of the total weight of said slurry.

2. A coating slurry for application to casting-defining surfaces of a foundry mold, said slurry consisting essentially of a liquid carrier and a dry blend, said dry blend consisting essentially of about 75% to 90% by weight of mica powder, about 4% to 14% by weight of corn cereal and about 3% to 8% by weight of wood flour, said liquid carrier being selected from the group consisting of methyl alcohol, ethyl alcohol, isopropyl alcohol, toluene, mineral spirits, naphthol spirits and water in proportions such that said dry blend constitutes approximately 15% to 25% of the total weight of said slurry.

3. A coating slurry for application to casting-defining surfaces of a foundry mold, said slurry consisting essentially of about 65% to 91% by weight of water and about 9% to 35% by weight of a dry blend, said dry blend consisting essentially of about 70% to 95% by weight of mica powder, about 2% to 20% by weight of corn cereal, about 1% to 12% by weight of wood flour and about 1% to 5% by weight of a nonionic, etherified polymeric carbohydrate, the particle sizes of said mica powder, corn cereal and wood flour not exceeding approximately -80 mesh, said slurry containing about 0.1% to 1% by weight of wetting agent.

4. A coating composition for application to casting-defining surfaces of a foundry sand mold, said composition consisting essentially of a suspension of a powder in water, said powder consisting essentially of, by weight, about 75% to 90% mica, 4% to 14% corn cereal and 3% to 8% wood flour, said suspension containing a polymeric organic binder in an amount not in excess of about 10% of the weight of said powder.

5. A foundry mold for use in producing a metal casting having at least one thin section, said mold being formed of foundry sand and having casting-defining surfaces provided with a thin coating consisting essentially of about 70% to 95% by weight of mica, 2% to 20% by weight of corn cereal and 1% to 12% by weight of wood flour.

6. A foundry mold for use in producing a metal casting having at least one thin section, said mold being formed of foundry sand and having casting-defining surfaces provided with a thin coating formed by applying to said surfaces a slurry consisting essentially of a liquid carrier and a dry blend, said dry blend consisting essentially of about 70% to 95% by weight of mica powder, about 2% to 20% by weight of corn cereal, about 1% to 12% by weight of wood flour and about 1% to 5% by weight of polymeric carbohydrate and a small amount of an antiflamentation agent, the amount of liquid carrier being sufficient to constitute about 65% to 91% of the total weight of the slurry.

7. A foundry mold for use in producing a metal casting having at least one thin section, said mold being formed of foundry sand and having casting-defining surfaces provided with a thin coating formed by applying to said surfaces a slurry consisting essentially of a dry blend suspended in a liquid carrier, said dry blend consisting essentially of about 75% to 90%, by weight, of mica powder, about 4% to 14%, by weight, of corn cereal, about 3% to 8%, by weight, of wood flour, the amount of liquid carrier in said slurry being sufficient to constitute about 65% to 91% of the total weight of said slurry, said liquid carrier being selected from the group consisting of methyl alcohol, ethyl alcohol, isopropyl alcohol, toluene, mineral spirits, naphthol spirits and water.

#### References Cited by the Examiner

##### UNITED STATES PATENTS

|           |         |                  |       |           |
|-----------|---------|------------------|-------|-----------|
| 1,858,083 | 5/1932  | Goldsmith        | ----- | 106—38.24 |
| 2,735,814 | 2/1956  | Hodson et al.    | ----- | 106—38.24 |
| 2,798,817 | 7/1957  | Lund             | ----- | 106—38.23 |
| 3,115,414 | 12/1963 | Lottridge et al. | ----- | 106—38.23 |

##### OTHER REFERENCES

"Webster's New International Dictionary," 2nd Edition, G. and L. Merriam Company, Springfield, Massachusetts, 1959, (page 725).

ALEXANDER H. BRODMERKEL, Primary Examiner.

JOHN R. SPECK, LESLIE H. GASTON, Examiners.